

March 19, 1935.

R. K. HOPKINS

1,994,649

PIPE COIL

Filed Dec. 20, 1932



Fig. 1



Fig. 2



Fig. 3

INVENTOR  
*Robert K. Hopkins*

BY  
*Virgil F. Davis*  
ATTORNEY

## UNITED STATES PATENT OFFICE

1,994,649

## PIPE COIL

Robert K. Hopkins, New York, N. Y., assignor to  
 M. W. Kellogg Co., New York, N. Y., a corpora-  
 tion of Delaware

Application December 20, 1932, Serial No. 648,957

5 Claims. (Cl. 196—133)

This invention relates to pipe coils and in particular to pipe coils of the character used in connection with the conversion, or cracking of high boiling point hydrocarbon oils to low boiling point hydrocarbon oils and similar processes.

In the cracking of petroleum oils, as at present practiced, it is not unusual to circulate fluids through pipe coils at pressures as high as 1100 pounds per square inch and at temperatures as high as 1100° F. Since the fluids circulated usually carry along with them solid particles, such as carbon, and contain corrosive impurities, such as sulphur, the diminution of the walls of the coils is rapid even at moderate velocities of flow of the fluids through the coils. The diminution or wearing away of the walls of the coils is believed to be caused by the combined effect of erosion, due to the entrained solid particles, and corrosion, due to the corrosive impurities of the fluids circulated. The diminution is appreciable throughout the coil but is especially noticeable at the headers connecting the straight lengths of the coils. Thus, in order to provide safe coils of reasonably long life it has become the practice to make the component parts of the coils out of special alloys such as tungsten-iron, chromium iron, etc., alloys. Coils made of these alloys are satisfactory, but very expensive.

I have found that I can obtain at least as satisfactory results as are obtained by the use of expensive alloys at only a fraction of the cost. In accordance with my invention I provide a coil the component parts of which are made up of carbon steel or similar material and have the surfaces normally exposed to the fluids circulated therethrough coated with a baked enamel of smooth glass like finish. Preferably I choose an enamel which is highly resistant to the corrosive components of the fluids circulated and which has a coefficient of expansion substantially equal to that of the steel of the coil. The resistant character of the enamel assures the corrosive effect due to the corrosive impurities in the fluid being kept at a minimum. Because of the smooth glass like finish of the enamel the resistance to flow through the coil is appreciably decreased with a consequent decrease in the turbulence at the headers. Since the finish is not only glasslike, but continuous and practically void of pores, pits etc., the tendency of the solid particles to accumulate on the walls and thus form eddy currents producing obstructions which are largely responsible for erosion, is reduced to a minimum also.

Other objects and advantages of my invention

will be best appreciated from a consideration of the following description taken together with the accompanying drawing in which,

Fig. 1 shows a side elevation of a pipe coil,

Fig. 2 is a sectional elevation taken on line 2—2 of Figure 3, and

Fig. 3 is a part sectional plan taken on line 3—3 of Figure 2.

The coil 10 is made up of a plurality of pipe lengths 11 connected by clamps 12 to goose neck 10 headers 13 to form the desired fluid path. The fluid circulated through coil 10 enters through pipe 14 and exits through pipe 15.

As best shown in Figures 2 and 3 pipes 11 are provided with flanges 16 at each end thereof. 15 Goose neck headers 13 are also provided with flanges 16 similar to those of pipes 11. Flanges 16 have circular grooves cut in their faces to accommodate therein gaskets 17. Each of clamps 12 comprises semi-circular pieces 18 and 19, having lugs at each end provided with holes 20 therein for the passage of bolts. The central inner portion of pieces 18 and 19 are cut away to provide semi-circular recesses adapted to house flanges 16. The arrangement is such that 25 when bolts 20 are tightened, the corners of the recesses of the pieces 18 and 19 move up on the incline faces of flanges 16 to force the flanges toward each other and by reason of gaskets 17 30 form a fluid tight joint. As shown by heavy lines 21, the surfaces of the pipe lengths 11 and goose neck headers 13 normally exposed to the fluid circulated through the coil 10 are coated with a baked enamel.

Pipe lengths 11 and goose neck headers 13 are 35 made of carbon steel or similar low priced metal and are formed to the desired size in accordance with the usual practice, the walls of pipe lengths 11 and goose neck headers 13 being made of the thickness necessary to withstand the pressures 40 for which coil 10 is designed and the inside diameter of pipe lengths 11 and goose neck headers 13 being made somewhat larger than called for in order to allow for enamel coating 21.

The inner surfaces of pipes 11 and goose neck 45 headers 13 as well as the faces of flanges 16, inside of the circular grooves which are adapted to accommodate gaskets 17, are then coated with frit. The frit chosen being such that it will 50 produce an enamel of smooth glass like finish, substantially devoid of holes, bubbles, pores and the like, and resistant to the corrosive action of the corrosion impurities of the fluid. The enamel produced also having a coefficient of expansion substantially equal to that of the carbon 55

steel, or other material, out of which pipe lengths 11 and goose neck headers 13 are made. The frit may be blown onto the surfaces to be coated in the powder form, or it may be applied thereto as a water suspension. After the frit has been applied pipes 11 and goose neck headers 13 are then allowed to stand until the frit is dried, after which the frit is brushed off or otherwise removed from any surface which it is not intended to enamel. 5 The coated parts of the coil 10 are then placed in a suitable furnace and subjected to temperatures ranging from 1300 to 1700° F. and are allowed to remain at these temperatures until the frit has fused and an enamel of proper character 10 has been produced. The parts are then removed from the furnace and the coil is ready for assembly. 15

It is to be noted that coil 10 made up of enameled carbon steel, pipe lengths 11 and goose neck headers 13 is in every way as strong as a similar coil made up of expensive alloy headers and pipe lengths. Furthermore, coil 10 is less subject to erosion and corrosion by reason of the 20 corrosion resistant qualities and the smooth glass like finish of the enamel. Also, since solid particles entrained in the fluid circulated through coil 10 do not have the tendency to stick to the glass-like surfaces of coil 10 the erosion due to eddy currents is practically eliminated. It is also 25 to be noted that because of enamel coating 21 the erosion and corrosion does not reduce the metal walls of coil 10. Hence when inspection shows that enamel coating 21 is badly worn a new enamel coating may be baked on and coil 10 30 made the equal in every way to a new coil. 35

I claim:

1. A pipe coil for cracking hydrocarbon under high pressure and heat, comprising a coil made up of a plurality of pipe lengths and header 40 means for connecting the ends of said pipe lengths to form a continuous fluid path, the inner surfaces of said pipe lengths and headers being coated with a corrosion resistant vitreous enamel having smooth glass like finish.
- 45 2. A pipe coil for cracking hydrocarbon under high pressure and heat, comprising a plurality of carbon steel pipe lengths, carbon steel header means for connecting the ends of said pipe lengths to form a continuous fluid path, the inner surfaces of said pipe lengths and said header means being coated with a baked on vitreous enamel of smooth glass-like finish, said enamel coating having a coefficient of expansion 50

substantially equal to that of the steel of said pipe lengths and said header means.

3. A pipe coil for cracking hydrocarbon under high pressure and heat, comprising a plurality of pipe lengths having flanges at each end thereof, header means having flanges at the ends thereof, adapted to cooperate with the flanges of said pipe lengths and means for connecting the flanges of said pipe lengths to the flanges of said header means to form a continuous fluid path, said pipe 10 lengths and said header means having the portions of their surfaces normally exposed to the fluid circulated through said coil coated with a corrosion resistant vitreous enamel of smooth glass like finish whose coefficient of expansion 15 is substantially equal to the coefficient of expansion of the material of said pipe lengths and said header means.

4. A pipe coil for cracking hydrocarbon under high pressure and heat, comprising a plurality 20 of parallelly arranged pipe lengths having flanges at each end thereof, headers having flanges at each end thereof, adapted to cooperate with said pipe lengths to form a continuous fluid path, packing means between the flanges of said pipe 25 lengths and the flanges of said headers, means for joining the flanges of said pipe lengths and the flanges of said headers in fluid tight relation, the surfaces of said pipe lengths and said headers defining the fluid path through said coil being 30 coated with a corrosion resistant vitreous enamel of smooth glass like finish whose coefficient of expansion is substantially equal to that of the material of said pipe lengths and said headers.

5. A pipe coil for cracking hydrocarbon under 35 high pressure and heat, comprising a plurality of parallelly arranged carbon steel pipe lengths having flanges at each end thereof, carbon steel headers having flanges at each end thereof adapted to cooperate with said pipe lengths to 40 form a continuous fluid path, packing means between the flanges of said pipe lengths and the flanges of said headers, and means for joining the flanges of said pipe lengths and the flanges of said headers in fluid tight relation, the surfaces 45 of said pipe lengths and said headers defining the fluid paths through said coil being coated with a corrosion resistant vitreous enamel of smooth glass like finish, whose coefficient of expansion is substantially equal to that of the steel 50 of said pipe lengths and said headers.

ROBERT K. HOPKINS.